

## 1

3,053,654

## PRODUCING LEAD SHAPES

Paul A. McKim, Baton Rouge, La., assignor to Ethyl Corporation, New York, N.Y., a corporation of Delaware

No Drawing. Filed Mar. 28, 1960, Ser. No. 17,802  
5 Claims. (Cl. 75—211)

This invention relates to the manufacture of lead shapes. More particularly, the invention relates to the preparation of solid lead shapes or articles from finely divided lead, or essentially lead systems, and especially lead systems derived from the preparation of organometallic compounds.

Although the general technique of forming solid shapes of metals from finely divided metals has been known for quite some time, it has been, for all practical purposes, not utilized for lead metal, probably because of the relatively low physical strength of the resultant product. It has recently been discovered that certain finely subdivided, essentially lead powders are highly suitable for making solid articles. These lead powders are derived from a reaction of an alkylating agent and an alloy of an alkali metal with lead, resulting in formation of a lead tetraalkyl compound plus unreacted subdivided lead powder. Such powders are highly effective sources of subdivided lead metal for forming purposes. It has been found that by mechanically forming such subdivided lead, that solid shapes having surprising rigidity, tensile strength, and other properties, can be readily made. Such forming operations necessarily must be preceded or followed by treatment to eliminate minor quantities of the lead tetraalkyl component present, such component being a residual quantity which is not normally removed from the reaction product mixture. The removal of such minor impurities, prior to a mechanical forming operation, is an inconvenient and relatively expensive operation. By this is meant that, although the tetraalkyl lead compound can be readily removed to a concentration low enough to satisfy the economics of production of the tetraalkyllead as a single product, considerable further treatment or effort is necessary to remove and recover the tetraalkyllead to the point that the ultimate lead shape is perfectly innocuous. Further, it has been discovered that the presence, of even minor quantities of liquid tetraalkyl compounds during a forming operation provides a beneficial effect in that such components appear to assist and facilitate the actual forming operation as such. The reasons for this are not fully understood, but the tetraalkyllead liquid components appear to have an oiliness and a lubricating effect which apparently minimizes the mechanical effort required to form solid shapes from such subdivided systems. Hence, the total elimination of tetraalkyllead compounds, before forming, is not a particularly satisfactory type of operation.

A general object of the present invention is to provide a new and improved process for the formation of solid lead shapes. More particularly, an object is to provide an improved process for forming lead shapes from finely divided lead residues from a process for making a tetraalkyllead compound, said process being characterized by the reaction of an alkylating agent with a lead alloy and an alkali metal. A more specific object is to provide a process producing lead solid shapes, employing the above mentioned feed solids wherein the benefits of minor quantities of copresent tetraalkyllead components, upon the forming operation, are fully preserved, yet the ultimate solid lead

## 2

shape is entirely freed of such materials. An additional object, of certain embodiments, is to provide a process wherein a portion only of a tetraalkyl component is removed and recovered and the solids, upon further processing are formed into desired solid shapes, and the remainder of the tetraalkyl is entirely eliminated. A more particular object is to provide in combination the synthesis of a finely divided lead solids system or mixture, and a forming operation for producing solid shapes therefrom.

10 Other objects will appear hereinafter.

The process of the present invention comprises subjecting a finely divided lead powder, consisting essentially of finely divided lead metal and accompanying minor quantities of tetraalkyllead compounds, to forming pressure operations at sufficiently elevated pressures to form the lead particles into an essentially homogeneous solid shape, and concurrently with said operation heating the lead particles and accompanying components to a temperature of from about 100° C. to about 300° C., for a time sufficient to essentially entirely thermally decompose the tetraalkyllead components. When moving pressures are utilized, the degree of movement can be varied and minimized by an appropriate increase in the forming pressure. In certain instances, entirely static pressures, i.e., with no movement of the lead powders other than that accompanying bulk volume reduction are employed. In virtually all cases, pressures of about 5000 pounds per square inch and above are employed. The duration of the temperature application will vary with the particular identity of the tetraalkyllead impurity or component, the concentration, and the intensity of temperature applied to the system during the processing. When lower temperatures, in the neighborhood of 100° or 150° are applied, and in the case of, for example, tetraethyllead, temperature applications of as high as an hour may sometimes be required, although usually 30 minutes is quite ample for most concentrations. On the other hand, when temperature levels of 200 to 300° C. are applied, the duration of such application can be as low as several seconds to about 10 minutes.

40 The general mode of operation, and the best manner of carrying out the invention, will be fully understood from the working examples and detailed description hereinafter.

## Example I

45 This example illustrates preparation of the charge stock for the present process by chemical means. 100 parts of monosodium lead alloy, NaPb, were charged to an autoclave along with about 50 parts of ethyl chloride, this amounting to approximately 75 percent excess ethyl chloride. The mixture was reacted at an autogeneous pressure at elevated temperature until the action was terminated, as shown by a decrease in temperature and pressure. The product of this reaction was an apparently dry reaction mixture containing about 55 weight percent lead, 24 percent tetraethyllead, and 20 percent sodium chloride. Excess ethyl chloride was vented during the reaction and upon completion of the reaction. The resultant dry granular material was then discharged from the autoclave and immersed in water, then was subjected to steam distillation for a sufficient period of time to remove a large proportion of the tetraethyllead component. The resultant material is a multiphase mixture of the subdivided lead particles, sodium chloride (largely dissolved in the aqueous phase) and minor quantities of tetraethyllead, in a concentration usually, of the order of several percent, based upon the lead.

Screening a portion of this material, in U.S. standard screens, gives the following size distribution:

| Cumulative Percent Retained | Screen No. | (Inches), Dimension of Screen Openings |
|-----------------------------|------------|----------------------------------------|
| 9                           | 18         | 0.0304                                 |
| 15                          | 25         | 0.0280                                 |
| 25                          | 35         | 0.0197                                 |
| 36                          | 45         | 0.0138                                 |
| 57                          | 100        | 0.0059                                 |
| 73                          | 120        | 0.0049                                 |
| 84                          | 200        | 0.0029                                 |
| 97                          | 325        | 0.0017                                 |

The lead powder, prepared as above described, is then fed to a rolling mill operation, being fed on a steel conveyor belt threaded through a pair of pressing rolls. Heating means, which are typically gas burners positioned below the steel belt, are provided slightly before the entrance to the rolling operation and provide sufficient heat to raise the temperature of the subdivided solids to about 250° C. In passing through the rolls, a pressure approximating 5000 pounds per square inch is applied, the actual time of contact between the rolls being about 1/30 minute. The duration of the temperature indicated, of the order of about 250° C., is about 3 minutes. A subsequent longer period is provided as the charge material is lowered in temperature to about 100°, this period requiring usually about 7 to 10 minutes. The indicated processing results in the formation of a thin lead strip, essentially free of tetraalkyl lead, and having very good surface gloss or finish, as well as being a stiff, sturdy material, having tensile strength of the order of 4000 to 6000 pounds per square inch. The degree of reduction of cross sectional thickness accomplished during the actual rolling is subject to easy adjustment. In typical operations, the average thickness of the lead powder feed stream is from about 1/6 to about 1/4 inch, and the pressing operation results in a thickness reduction of from 50 to 90 percent, a typical sheet having a thickness of about 0.04 inch.

#### Example II

In this example, the same feed supply is used, as in Example I, but instead of rolling the lead powder, it is charged to an elongated cylindrical extrusion chamber, having a die at one boundary thereof, the chamber and die providing an extrusion ratio of the order of 42. The die is in the shape of a cylindrical or circular aperture of about 0.4 inch in diameter. Pressure of about 25,000 pounds per square inch is applied. Concurrently with applying the pressure, the extrusion chamber is heated by external means, typically a resistance wire winding, or in some cases, an induction heating coil, to heat the chamber and the contents to about 175° C. Upon application of pressure to the charge, by a ram in the extrusion chamber, a substantially homogeneous, cylindrical shape is forced through the die, at a temperature approximating

about 5 minutes. A finely grained lead solid, virtually free of tetraethyllead, is produced. In preferred embodiments of this example, the temperature gradient is applied so that a higher temperature is provided at the extrusion end of the chamber and lower temperatures are applied in the chamber proper. This technique provides the benefit of retaining the alkyl lead or tetraethyllead component unchanged during a large portion of the processing, and thus assures a lubricating effect derived from the tetraethyllead component. The accompanying water with the charge stock is concurrently vaporized from the system and is removed by blowby past the ram, and to a certain extent by vaporizing through the die apertures.

In addition to rolling and extrusion as exhibited in the above examples, the forming operations employed include direct pressing of the lead powder charged in a press mold or die having a desired final part configuration, which can be, for example, forms for radiator ornaments, name plates, parts for railroad and ship models, and other articles. The following example illustrates the technique employed in such instances.

#### Example III

Again the powder employed is as in Example I and specimens of this powder are inserted in a die or mold providing a cylindrical bushing pattern. Pressure is applied thereto by a mating ram, at a pressure of about 25,000 pounds per square inch. Concurrently the mold is heated to a temperature of 115° C. and pressure and temperature are maintained for approximately 15 minutes. At the termination of this period, the formed bushing is discharged from the mold, and has smooth surfaces and sharp configurations. Analysis of a fragment broken from the shape shows virtually no detectable organolead component.

#### Example IV

In this operation, the lead powder was derived generally as obtained in the preceding examples, but the composition thereof differed in that it contained approximately 6 weight percent tetraethyllead and about 11 percent water. The material was charged to an extrusion chamber, and a pressure of about 15,000 pounds per square inch is applied, employing an extrusion ratio of about 35. The extrusion chamber and contents are heated to a temperature of about 190° C., resulting in rapid decomposition of the tetraethyllead component and vaporizing of the water phase, which was discharged in part as a vapor discharged backwards past the extrusion ram and to a minor extent, by concurrent discharge through the die orifice. The residence time of the material in process, in the extrusion chamber, is about 3 minutes, and approximately 5 to 10 minutes additional time is required for the solid lead product to cool to a temperature of below 100° C. The product is a dry, substantially homogeneous bar, having virtually no tetraethyllead as such therein.

In addition to the foregoing operations, additional working examples are summarized in the following table:

| Example | Composition of Feed  |             |                             | Forming and Treating |                   |                  |                            |
|---------|----------------------|-------------|-----------------------------|----------------------|-------------------|------------------|----------------------------|
|         | Alkyllead            | Wt. Percent | Size of Solids <sup>1</sup> | Technique            | Pressure (p.s.i.) | Temperature, °C. | Duration <sup>2</sup> Min. |
| V       | Tetra-n-butyl lead   | 5           | Through 100- on 200         | Rolling              | 4,000             | 140              | 2                          |
| VI      | Tetra-1 Propyl lead  | 5           | Through 100- on 325         | Extrusion            | 10,000            | 130              | 4                          |
| VII     | Tetra-isooamyl lead  | 7           | Through 35, on 100          | Pressing             | 28,000            | 110              | 7                          |
| IX      | Methyl-triethyl lead | 2           | Through 18-----             | do                   | 17,000            | 130              | 8                          |
| X       | Dimethyl-diethyl     | 1.5         | Through 18-----             | Rolling              | 15,000            | 130              | 3                          |
| XI      | Methyl-triethyl lead | 0.5         | Through 18-----             | Extrusion            | 20,000            | 140              | 5                          |

<sup>1</sup> Screen numbers refer to U.S. Sieve Series.

<sup>2</sup> Refers to time under pressure or in processing; additional time also required in cooling to below 100° C.

175° C. The duration of residence time in the extrusion chamber and the die is up to about several minutes, and the formed lead shape retains the temperature, or a temperature of about 100° C. for an additional period of

As heretofore mentioned, the present forming operations can be carried out in conjunction with preceding recovery operations of similar character. In other words, an intermediate forming operation is directed to a partial

removal of a co-present tetraethyllead, providing an intermediate solid shape having appreciable quantities of alkyl lead therein, and such shape is then further mechanically shaped by pressure application concurrently with thermal decomposition as in the preceding examples. An illustration of such embodiment follows.

*Example XII*

A reaction mixture is prepared by reacting sodium lead alloy and ethyl chloride, as in Example I. Only a portion of the tetraethyllead is removed by steam distillation, however, reducing the concentration thereof to about 15 percent of the lead.

The solids containing residue is free drained leaving a wet powder containing mixture with the indicated proportions of tetraethyllead and comparable amounts of aqueous phase. Portions of the mixture are pressed at ambient temperature. This initial pressing is in a cylindrical chamber, by application of pressure by a ram. Sufficient clearances are provided to allow discharge of liquid phases past the ram or plunger. Upon application of pressure of about 5000 pounds per square inch, a solid appearing shape is formed, having roughly about 3 weight percent tetraethyllead and comparable proportions of water or aqueous phase.

The solid shapes, as above formed, are then charged to an extrusion chamber and processed as in Exhibit II, except that the extrusion orifice in this instance is in the form of a thin strip shape. As in preceding examples, this operation is accompanied by heating to a temperature of, typically 150° C., to provide complete decomposition of the tetraethyllead content.

It will be apparent from the foregoing examples that the principles of the present invention are applicable to a substantial number of particular systems, and that a variety of forming techniques can be employed.

As evident from the examples, in all instances a substantial temperature of above 100° C. and below about 300° C., is employed for the process. The decomposition of the alkyl lead compounds varies in rapidity according to the particular identity of the particular alkyl lead and according to certain other factors, e.g., concentration. In the case of tetraethyllead, measurable decomposition occurs in the neighborhood of 100° C., but the rate is quite low, particularly when minor quantities of thermal decomposition inhibitors are present in solution in a solution in a tetraethyllead. Ordinarily then, and particularly because of a supplemental stabilizing effect of solids present, a temperature of above about 130° C. is preferred for this particular material. However, temperatures, as indicated, of the order of above 110 or 115° C. are quite suitable and if the temperature level is maintained for a sufficient period of time, full decomposition of the organolead material is accomplished. The tetraalkyllead compounds having alkyl groups of more than two carbon atoms are more easily decomposed than the tetraethyllead. Tetramethyllead, on the other hand, is quite refractory in its resistance to thermal decomposition, and when this is the component present, temperatures approaching the range of about 290 to 300° C. are ordinarily preferred to accomplish this result.

The alkyl lead compounds, under the conditions of the present process, do not decompose violently. It appears that the relatively large proportions of lead solids, plus the co-presence, usually, of an aqueous phase, results in a distinct moderation of the potential severity of decomposition. Although alkyl lead compounds with higher alkyl substituents are more readily decomposed, the compounds with lower alkyl substituents are more apt to exhibit violent decomposition. Hence, in the case of the latter, it is highly preferred that the alkyl lead concentration should not exceed about 5 percent.

The time necessary to process and maintain temperature during the processing at the desired level necessary for decomposition, will depend to some extent upon the

proportions of the alkyl lead compound, upon its identity, and by the temperature level applied. Heating and cooling periods, to and from the highest temperature of a process, also contribute to the decomposition. The overall processing times, in which temperatures of over 100° C. prevail, are usually from 1 to 15 minutes. However, by increasing the temperatures during actual pressure forming operations, the necessary pressure period can be drastically reduced. Thus, by increasing the maximum temperature, during Example III, to about 200° C., the pressure application period can be reduced to several seconds. Similar reductions in time are attainable in the other examples.

The actual pressures employed in forming the lead shapes will depend upon the degree of compacting actually desired and the mode or technique employed in the forming. As clear from the above examples, suitable pressure ranges are from the range of several thousand to about 30,000 pounds per square inch, although these are not explicitly limiting. A preferred range is from about 10,000 to about 20,000 pounds pressure.

The particular weight concentration of the lead alkyls is not highly critical. It is preferred that the lead powder feed contain not over about 5 weight percent of the alkyl lead component, but the process is equally operable with higher concentrations of the order of 7 or even up to about 10 weight percent. In these instances, a portion of the alkyl lead component is actually dislodged from the feed material under the influence of the pressure alone, and may be recovered as such. When the concentration is of the order of about 1.5 or 1 percent or lower, virtually all the removal of the alkyl lead is by the mechanism of thermal decomposition as above described.

Having fully described the invention in the several modes of operation, what is claimed is:

1. The process for forming solid lead shapes comprising forming, by application of pressure of at least about 5,000 pounds to about 30,000 pounds per square inch, a solid shape from a finely divided predominantly lead powder, said powder consisting essentially of finely subdivided lead and from about 0.5 to 10 weight percent of a tertiakyllead compound, and concurrently with said pressure forming operation, heating to a temperature of above about 100 to about 300° C. for a time sufficient to thermally decompose the tertiakyllead compound.
2. The process of claim 1 further defined in that the pressure is static pressure applied to the lead powder in a forming die.
3. The process of claim 1 further defined in that the pressure is applied to the lead powder by forming rolls.
4. The process of claim 1 further defined in that the lead powder is charged to an extrusion chamber and pressure is applied to force a solid shape through a forming die in the boundary of said chamber.
5. The process comprising, in combination, reacting an alkali metal lead alloy with ethyl chloride, forming thereby a reaction product including tetraethyllead, excess lead in finely divided form, and alkali metal chloride, separating substantially all the alkali metal chloride and the preponderance of the tetraethyllead therefrom, thereby forming finely subdivided lead powder accompanied by minor quantities of from about 0.5 to 5 percent of tetraethyllead, then subjecting said powder to a forming operation including application of pressure of at least 5,000 pounds per square inch and concurrently heating to a temperature of above about 100° to about 300° C. for a time sufficient to thermally decompose the tetraethyllead, whereby a solid shape substantially free of tetraethyllead is produced.

References Cited in the file of this patent

UNITED STATES PATENTS